

# UNITED STATES PATENT OFFICE.

JAMES M. CORDRAY, OF LOS ANGELES, CALIFORNIA.

## COMPOUND FOR IGNITING BLAST-FUSES.

1,072,827.

Specification of Letters Patent. Patented Sept. 9, 1913.

No Drawing.

Application filed January 24, 1912. Serial No. 673,251.

*To all whom it may concern:*

Be it known that I, JAMES M. CORDRAY, citizen of the United States, residing at Los Angeles, in the county of Los Angeles and State of California, have invented certain new and useful Improvements in Compounds for Igniting Blast-Fuses, of which the following is a specification:

This invention has as its object to provide a compound to be applied to blast fuses to insure their ignition.

In blasting, it is customary to fire several charges at a time and it not infrequently happens that one or several charges will fail to be ignited due to the fuse becoming extinguished. When this occurs, a miner is liable to drill into the unexploded blast with disastrous results. The failure of the fuse to burn is usually due to the fact that its end which is ignited, rests upon a damp spot or the flame is not held to it for a sufficient length of time to insure of its becoming properly ignited.

The present invention therefore aims to provide a compound which is to be applied to the end of such a fuse immediately prior to igniting the same, which compound will cause proper ignition of the fuse even though it be damp or has previously been dipped in water.

The compound of the present invention is composed of the following ingredients in substantially the quantities stated:

|    |                      |         |
|----|----------------------|---------|
| 35 | Powdered gum camphor | 1½ ozs. |
|    | Oil of sassafras     | ½ oz.   |
|    | Potassium nitrate    | 1 oz.   |
|    | Oil of eucalyptus    | 4 ozs.  |
|    | Kerosene             | 12 ozs. |

40 In mixing the compound there is placed in a suitable receptacle one-half ounce of oil of sassafras, one ounce of powdered potassium nitrate, four ounces of oil of eucalyptus, and one-half ounce powdered camphor. 45 The receptacle is then placed in a water bath and heated. The water bath should preferably be arranged to cover about two-thirds of the exterior surface of the said receptacle. The ingredients within the receptacle are

first heated to a temperature of 150° F. and are stirred for about a minute. The contents of the receptacle are then emptied into another receptacle and cooled to 100° F. To the mixture thus cooled there are added twelve ounces of kerosene and after the mixture has been thoroughly stirred it is poured into suitable cans and the cans are sealed until the mixture is to be used in the mine.

50 In using the compound, that end of the fuse which is to be ignited, is dipped into the compound and is split for a distance, preferably for about one-half inch of its length. The end of the fuse is then ignited and the compound with which it has been 55 saturated will burn for a sufficient length of time to insure of proper ignition of the remainder of the fuse.

60 I employ gum camphor in my fuse igniting compound for the reason that this substance will burn with a steady flame without emitting sparks and will take fire readily even though it has been dipped in water. The oil of sassafras and oil of eucalyptus are employed for the purpose of retaining 65 the strength of the camphor and preventing its evaporation and also for the reason that the oil of eucalyptus is highly inflammable. The coal oil is used to render the compound 70 of proper consistency for use and also for 75 the reason that it is inflammable.

Having thus described the invention what is claimed as new is:—

1. A fuse igniting compound including 80 potassium nitrate, gum camphor, and kerosene.

2. A fuse igniting compound consisting of 85 gum camphor, potassium nitrate, oil of sassafras, oil of eucalyptus, and kerosene.

3. A fuse igniting compound including a 90 mixture of potassium nitrate, gum camphor, and a liquid hydrocarbon.

4. In testimony whereof, I affix my signature in presence of two witnesses.

JAMES M. CORDRAY. [L. S.]

Witnesses:

ALVIN GALLAHER,  
MARY A. CORDRAY.